

## UNITED STATES PATENT OFFICE

WALTER H. PFEIL, OF READING, PENNSYLVANIA, ASSIGNOR TO BIRDSBORO STEEL FOUNDRY AND MACHINE COMPANY, OF BIRDSBORO, PENNSYLVANIA, A CORPORATION OF PENNSYLVANIA

## CHILLED IRON ROLL

No Drawing.

Application filed January 5, 1932. Serial No. 584,901.

My invention relates to chilled cast iron rolls for use in rolling mills and it has for its general object to provide a chilled roll consisting of an iron alloy of a composition such that chilled rolls made thereof will have greater strength, greater hardness, better wearing qualities and greater resistance to fire cracking than the ordinary chilled cast iron rolls heretofore in use.

10 A further characteristic of a chilled iron roll consisting of an alloy embodying my invention is that deep grooves may be formed therein without the excessive depth of chill which is required in the case of ordinary chilled rolls.

A further purpose is to make a chilled cast iron roll containing chromium and copper, and at the same time to avoid the undesirable characteristics imparted to the roll by 20 effective quantities of molybdenum.

A further purpose of my invention is to form a chilled roll of an iron alloy having a carbon content within the cast iron range, containing an effective amount of chromium but not more than 2.00%, an effective amount of copper but not more than 1.50%, and no molybdenum or at least not more than .10% of molybdenum.

In the present day practice in rolling mills, chilled cast iron rolls are subjected to great stresses and strains and altogether undergo very hard usage. Heretofore this condition has been met in some cases by increasing the sizes of the rolls in order to obtain the requisite strength and in others by the employment of very expensive alloys. But this is objectionable and it is highly desirable to obtain the requisite strength and ruggedness without the necessity of increasing the dimensions or sizes of the rolls and without the employment of very expensive alloys.

By my invention I am enabled to employ rolls of smaller diameter, to perform certain kinds of work, than would be required if ordinary chilled rolls were employed. In other words, I am enabled to perform work on smaller mills that otherwise would require the use of larger and more expensive mills.

It is a further purpose of my invention to provide a chilled cast iron roll in which the primary or outer chill is very thin; that is to say, is very light and merges into the secondary or inner chill without any appreciable line of demarcation. By providing chilled rolls with this characteristic feature of construction, I am enabled to provide deep grooves in the same for the purpose of giving the shapes desired to beams, rods and the like, which are passed between adjoining rolls, without the requirement of a great depth of chill, such as is required in ordinary chilled rolls for this kind of work. The composition of the ferrous alloy referred to herein is such as to make possible the production of a chilled cast iron roll having the characteristic qualities above mentioned.

Further purposes appear in the specification and in the claims.

This application is intended to embody the entire subject matter of my application now pending, for chilled iron rolls, Serial No. 431,635, filed February 26, 1930.

In a roll having the composition of my invention, the surface hardness and hardness of metal toward the center of the roll differ but slightly. However, there is a gradual decrease in hardness, the hardness of the outer surface portion of the roll merging gradually into the secondary chill and interior portion of the roll, as already indicated. Thus a homogeneous, dense and very strong structure is produced, due primarily to the new composition employed by me in the manufacture of my roll.

In the manufacture of ordinary chilled iron rolls, it heretofore has been the practice to employ silicon, manganese, sulphur, phosphorus, carbon and iron, the percentages of these materials varying with the character of roll desired. My reference to the character of roll desired is meant to refer to the character of work for which the roll is to be employed.

It may be noted that the mixture of pig iron, scrap and alloys used in the manufacture of chilled iron rolls is usually melted in an air-furnace, but might also be made by

the use of an open-hearth, electric or cupola furnace.

Attempts have previously been made to produce chilled cast iron rolls using chromium, from .25 to 3.50%; copper, from .25 to 2.00%; and molybdenum, from .10 to 2.00% in addition to non-effective quantities of the various metalloids. I have discovered that, by eliminating the molybdenum here-<sup>5</sup>tofore considered essential, a much superior roll may be produced, having the characteristics of increased strength, hardness, wearing qualities and power to resist fire cracking.

By eliminating molybdenum, I do not mean that it must be altogether absent, and in fact in the normal case some very small quantity of molybdenum will be present in the roll of my invention, due to the almost inevitable presence of molybdenum in the scrap. I <sup>10</sup>mean to imply, however, that molybdenum will not be present in an effective quantity, that is, that its percentage will not rise above a fraction of .10%.

I find that rolls made in accordance with my invention may have very deep grooves without the necessity for excessive or great depth of chill, as has been required in the prior art.

Chilled rolls of ordinary cast iron lack the strength necessary to enable them to perform many kinds of work which they are called upon to perform. This is particularly true where very deep chill is required.

My roll produced by the use of chromium and copper, without effective quantities of molybdenum, has been found by me to be much superior to the same roll containing the chromium and copper along with an effective quantity of molybdenum.

The molybdenum tends to cause the precipitation of graphitic carbon in the chilled section of the roll. It appears that the presence of molybdenum undesirably favors the reaching of equilibrium during chilling; <sup>40</sup> in other words, molybdenum opposes the formation of the "grain" structure which is most desirable in rolls of this type. Due to the grain visible in photomicrographs of the chilled sections of rolls of the kind to <sup>45</sup> which I am referring, such rolls are commonly known in the trade as "grain" rolls.

I therefore find it most desirable to preserve the grain structure in its most pronounced form by omitting molybdenum in <sup>50</sup> effective quantities.

Where molybdenum is not present in effective quantities, the grain structure is not only more pronounced, but it is also more uniform and more homogenous in the chilled section.

Frequently during the casting of rolls, cracks and incipient cracks develop which either cause rejection of the casting at the foundry or else lead to failure in service and ultimate replacement.

Where molybdenum is present, the tend-

ency of the roll to crack is thereby increased. I have observed that the percentage of rejections of castings has decreased markedly in instances where effective quantities of molybdenum have been omitted, as compared with those cases in which effective quantities of molybdenum have been used.

From the standpoint of furnace practice and casting, it will be obvious, and it is the actual experience, that the alloy containing the four effective components iron, carbon, chromium, and copper is much more easily handled than the five component alloy having the additional element molybdenum in effective percentage.

An additional feature of wide commercial importance is the lower cost of my roll as compared with the roll in which molybdenum is used. By avoiding the use of effective quantities of molybdenum, I avoid the need for the most costly alloy ingredient of the three components chromium, copper and molybdenum. For example, on the basis of the alloy ingredient the cost of molybdenum is approximately \$1.00 per pound, as against 15¢ per pound for chromium and 9¢ per pound for copper. Furthermore, I find that the percentages of chromium and copper need be no higher when molybdenum is absent than when it is present.

In effect, I have discovered that the molybdenum, which was formerly considered highly desirable in "grain" rolls, is in fact a deleterious ingredient if it is present to an extent of more than .10%. All of the advantages previously attributed to the molybdenum in the combination may be obtained by using the chromium and copper alone in the cast iron.

In making up my alloy I ordinarily charge the furnace with scrap and also with pig iron. The scrap, especially when obtained from previously used rolls of a type not embodying my invention frequently contains a relatively high content of molybdenum, as for example, .50% or more, and I therefore dilute this high molybdenum scrap by melting with it or adding to it pig iron or other ferrous material low in molybdenum or lacking in molybdenum. In this manner the total molybdenum content of the resultant molten charge will be below that which is considered an effective quantity of molybdenum.

A certain oxidation of oxidizable ingredients present in the charge, such as chromium, is inevitable during melting and during furnace operation. I therefore find it necessary to add chromium even when the chromium content of the charge as calculated from the content of the solid raw materials was initially correct. I also find it necessary in most cases to add copper to enrich the charge. During the additions of alloying ingredients, especially chromium and copper, I am care-

ful to avoid any addition of molybdenum, as I desire to limit the molybdenum content to the lowest amount consistent with the use of the scrap available. For convenience I 5 have referred to additions of copper and chromium from the standpoint of the enrichment of the charge in these metals. My alloy as prepared in my furnace is primarily intended for casting and chilling, since its composition 10 is controlled by my desire to avoid the possibility of cracks during casting and chilling and of subsequent cracking during service. I find the alloy disclosed well suited to form a thin surface chill and that there 15 is less danger of cracking with a thin chill and a progressively changing backing than with a thick chill with dependence upon the thickness of the chill in that event, rather than the flexibility.

20 The percentage of copper and chromium to be used vary or differ for different sizes and kinds of rolls. As already suggested, it is meant by "kinds" of rolls to refer to the nature of the work it is expected that they 25 shall be required to do.

In the production of an alloy in accordance with my invention I propose to employ the ingredients heretofore indicated, including chromium and copper, in percentages 30 somewhat as follows:

|            |                |
|------------|----------------|
| Carbon     | 2.50% to 4.00% |
| Chromium   | .75% to 2.00%  |
| Copper     | .25% to 1.50%  |
| Molybdenum | 0.00% to .10%  |
| Silicon    | .50% to 2.00%  |
| Manganese  | .25% to 1.25%  |
| Sulphur    | .025% to .20%  |
| Phosphorus | .025% to .50%  |

40 the remainder sufficient to make up 100% consisting of iron.

As has been indicated previously herein the percentages of the ingredients enumerated may be varied in order to produce rolls 45 having characteristics which will best fit them for operations under the conditions heretofore indicated.

It may be noted that the casting of rolls of a composition embodying my invention is 50 carried out in the manner usually employed in the casting of ordinary chilled rolls, chill pass, and rolls in which condensing chills are used; hence it is deemed unnecessary to refer in detail to the manner or way in which 55 the casting operation is performed.

I desire to get the full benefit of the copper and chromium ranges of content indicated, which are of real value but which have been clouded in previous teachings by effective 60 and therefore objectionable contents of other ingredients, of which one of the most objectionable is molybdenum.

By reason of the very powerful effect of molybdenum as an alloying ingredient, even 65 a small quantity of molybdenum becomes

effective and therefore objectionable. For example, in a previous alloy the good effects of the presence of copper and chromium have been negated by the presence of an effective quantity of molybdenum, indicated as being 70 present in as low a quantity as .10%. It will be evident that the benefit of my invention is to be measured by maintenance of the content of molybdenum below that which becomes effective, rather than upon any given and 75 definite percentage of molybdenum. My own experience agrees with the teaching of the prior art that molybdenum to be effective must be approximately .10%.

In view of my invention and disclosure 80 variations and modifications to meet individual whim or particular need will doubtless become evident to others skilled in the art, to obtain part or all of the benefits of my invention without copying the structure 85 shown, and I, therefore, claim all such in so far as they fall within the reasonable spirit and scope of my invention.

Having thus described my invention, what I claim as new and desire to secure by Letters 90 Patent is:

1. A chilled cast iron roll wherein there is no distinct line of demarcation between the primary chill and the secondary chill, containing 95 between 0 and .10% of molybdenum and comprising as essential ingredients of the composition thereof chromium and between about .75% and 2.00% and copper between about .25% and 1.50%.

2. A chilled cast iron roll containing and 100 comprising as essential ingredients in the composition of the material of which the roll consists chromium and copper, the percentage of chromium ranging from about .75% to not more than 2.00% and the percentage 105 of copper ranging from about .25% to about 1.50% and containing less than .10% of molybdenum.

3. A chilled cast iron roll for rolling metals 110 wherein the outside primary chill is thin and merges into the secondary chill without any appreciable line of demarcation and wherein also the surface hardness and hardness of the metal toward the center of the roll differ but slightly, containing between 0 and 115 .10% of molybdenum and comprising as essential ingredients chromium which may range from about .75% to about 2.00% and copper which may range from about .25% to about 1.50%, the said roll being further characterized in that it offers relatively great resistance to fire cracking.

4. A chilled cast iron roll wherein the outside primary chill is thin and merges into the secondary chill without any appreciable line 125 of demarcation and wherein also the surface hardness and hardness of the metal toward the center of the roll differ but slightly, the composition of which consists of carbon which may range from about 2.50% to about 130

4.00%, chromium from about .75% to about 2.00%, copper from about .25% to about 1.50%, molybdenum from 0% to about .10%, silicon from about .50% to about 2.00%,  
5 manganese from about .25% to about 1.25%, sulphur from about .025% to about .20%, phosphorus from about .025% to about .50%, and iron sufficient to make a total of 100%.

5. A chilled cast iron roll characterized in  
10 that the surface thereof is hard, dense and resistant to abrasion and in which the said surface portion merges gradually into the inner portions of said rolls without a definite line of demarcation, the said roll offering relatively great resistance to fire cracking, containing between 0 and .10% of molybdenum and comprising and containing as essential ingredients in its composition chromium and copper, the former in proportions which may  
15 range from .75% to about 2.00% and the latter in proportions which may range from about .25% to about 1.50%, the presence of the specified characteristics of said roll being due to the casting thereof against a chilling  
20 medium.

WALTER H. PFEIL.

30

35

40

45

50

55

60

65